

## UNITED STATES PATENT OFFICE

2,500,162

METHOD OF PREPARING VISCOS OILS BY  
THE THERMAL CONDENSATION OF SHORT  
CHAIN MONOOLEFINS WITH LONG CHAIN  
MONOOLEFINS

Francis M. Seger, Pitman, and Alexander N. Sachanen, Woodbury, N. J., assignors to Socony-Vacuum Oil Company, Incorporated, a corporation of New York

No Drawing. Application September 2, 1948,  
Serial No. 47,556

11 Claims. (Cl. 260—683.1)

1

This invention has to do with a new and novel class of synthetic lubricants and with a method for preparing the same. More particularly, the invention has to do with synthetic lubricants characterized by an especially desirable combination of properties, namely, low pour point, high viscosity index and excellent stability.

As is well known in the art, considerable attention has been given to the development of synthetic lubricants from various sources, particularly olefinic hydrocarbons. For example, olefins have been polymerized in the presence of numerous catalysts, notably those of the Friedel-Crafts type, whereupon viscous oils have been formed. In the absence of catalysts, however, olefins as a class have not been so successfully converted to viscous oils. Ethylene has been found to be unlike most low molecular weight olefins, in that it may be converted under high pressure and at elevated temperatures of the order of 500-750° F., in the absence of active catalysts, to high viscosity index lubricants. Other low molecular weight olefins such as propylene and butenes, which are normally gaseous in character, do not produce lubricating oils on thermal (non-catalytic) treatment. Oils obtained from propylene, butenes and pentenes, in the absence of active catalysts, are formed in only low yields and have undesirable properties, in particular, low viscosity indices. Longer chain olefins—other than normal, alpha mono-olefins having six or more carbon atoms—have also failed to form desirable viscous oils in appreciable quantities when thermally polymerized and condensed. Typical of such olefins are pentene-2, octene-2 and 2-ethyl hexene-1. With still longer chain olefins such as those having about twenty or more carbon atoms, substantial yields of synthetic oils of high viscosity indices have been realized; yet, such oils have excessively high pour points.

In application Serial No. 761,716, filed July 19, 1947 by applicants and now abandoned, and of which this application is a continuation-in-part, disclosure was made of the discovery that normal, alpha mono-olefins having from six to twelve carbon atoms can be converted by thermal, non-catalytic treatment under controlled reaction conditions to excellent synthetic lubricants. It has now been discovered that short chain and long chain mono-olefins can also be converted by thermal and non-catalytic treatment to similarly characterized synthetic oils.

The present invention is predicated upon the discovery that synthetic oils having low pour points, high viscosity indices and excellent stability are formed in a thermal, and non-catalytic, treatment of a mixture of a short chain mono-olefin and a relatively long chain normal, alpha mono-olefin, said mixture being properly proportioned such that the mean value of the olefin

2

chain length falls within the range of six to twelve carbon atoms. Thus, the present invention makes possible for the first time the use of inexpensive short chain mono-olefins for the production of synthetic lubricants, by thermal means. In this way, then, readily available commercial materials may be used, thereby lowering the cost of raw materials and hence the ultimate cost of the product. For economically practical operation on a commercial basis, mixed olefinic materials of relatively long chain length such as those obtained from cracked hydrocarbon waxes or cracked paraffinic distillates, and from Fischer-Tropsch and related processes, constitute desirable sources of raw materials.

## Reactants

The short chain mono-olefin reactant used herein is one having from 2 to 6 carbon atoms per molecule. Typical of such olefins are ethylene, propylene, butene-1, butene-2, isobutylene, pentene-1, pentene-2, hexene-1, hexene-2, hexene-3, etc. Inasmuch as the normal, alpha mono-olefins of this group form outstanding synthetic lubricants with the long chain normal, alpha mono-olefins (defined below), they represent preferred short chain mono-olefins. It will be understood, of course, that individual mono-olefins of the foregoing group may be used, and that mixtures of two or more of such short chain mono-olefins may be used.

As indicated above, the other mono-olefins used in forming the synthetic lubricants of this invention are long chain normal, alpha mono-olefins containing from 10 to 30 carbon atoms per molecule. In some instances, the mono-olefin may contain as many as 30 carbon atoms per molecule. Preference is given, however, to those falling within the range of 12 to 20 carbon atoms per molecule, such preference being based upon the outstanding lubricants obtained therefrom in association with the foregoing short chain mono-olefins. Illustrative of long chain normal, alpha mono-olefins are the following: decene-1, undecene-1, dodecene-1, octadecene-1 and the like. It will be clear from the foregoing examples that an alpha olefin may also be referred to as a 1-olefin.

Not only may the long chain mono-olefins of the aforesaid character be used individually in this invention, but they may also be used in admixture with each other. In addition, olefin mixtures containing a substantial proportion of such long chain mono-olefins may be used with the short chain olefins. Preferred of such mixtures are those containing a major proportion of a 1-olefin or 1-olefins. In general, such mixtures should preferably contain not more than about 20% by weight of hydrocarbons other than straight chain 1-olefins of the type described. In

the practice of this invention, however, it has been found that charge stocks containing as much as 50% by weight of paraffinic hydrocarbons, with the balance straight chain 1-olefins, are definitely usable. Representative of such mixtures are those obtained by cracking of paraffin waxes and other paraffin products, and those obtained from the Fischer-Tropsch and related processes. The latter mixtures may contain, in addition to the 1-olefin or 1-olefins, such materials as: other olefins, paraffins, naphthenes and aromatics.

In many instances, in commercial operation, it will be found desirable to use technical grades of 1-olefins. Mixed olefinic materials derived from thermal cracking of hydrocarbon wax or from the Fischer-Tropsch process constitute satisfactory charging stocks, with the short chain olefins. In this connection, it must be noted that it is suspected that substantially straight chain 1-olefins, i. e., 1-olefins in which the length of the side chain or chains is short relative to the length of the main chain, are also suitable, although less advantageous charge stocks for the purpose of the present invention. In view of the unavailability of such olefins, however, no test data can be adduced to confirm this suspicion.

#### Reaction conditions

The most critical reaction conditions, coupled with the specific character of the aforesaid reactants, are the proportion of the reactants and the temperature of reaction.

As indicated previously, the short chain mono-olefin having from 2 to 6 carbon atoms and the long chain normal, alpha mono-olefin are reacted in such molar proportions that the mean value of the olefin chain length in the reaction mixture is from about 6 to about 12 carbon atoms. In other words, one molar proportion of ethylene, 2 carbon atoms, may be suitably reacted with one molar proportion of hexadecene-1, 16 carbon atoms, for the mean value of the olefin chain length of the original reaction mixture is then nine carbon atoms. Similarly, one molar proportion of isobutylene, four carbon atoms, and one molar proportion of octadecene-1, 18 carbon atoms, form a reaction mixture of the character contemplated herein; in this case, the mean value is eleven carbon atoms. By way of further illustration, two molar proportions of propylene, 3 carbon atoms, and one molar proportion of tetradecene-1, 14 carbon atoms, form a suitable reaction mixture, with a mean value of 6.7. Particularly outstanding synthetic lubricants are formed when the mean value of the original reaction mixture is about 10.

With regard to reaction temperature, it has been found that this factor should be maintained within the range of from about 500° F. to about 750° F. Most satisfactory results, however, are obtained when operating within the more limited range between about 600° F. and about 700° F. Operation under the latter conditions makes possible synthetic lubricants of outstanding quality, in satisfactory, commercially feasible yields.

At temperatures between about 500° F. and 600° F., conversion of the olefin reactants to synthetic lubricants takes place at a slower rate and is usually less complete. At temperatures greater than 700° F., side reactions and secondary reactions begin to occur, and increase in importance to such an extent that at temperatures above about 750° F., the process becomes impracticable. These side reactions and secondary reactions are chiefly the following:

(1) The volatile, non-oily components of the reaction mixture become progressively more saturated, as indicated by a decrease in bromine addition number and, therefore, less suitable for recycling for further conversion;

(2) Cracking begins, as evidenced by gas pressure and decrease in oil yields; and

(3) Cyclization begins, as evidenced by some decline in viscosity index with accompanying increase in gravity and refractive index.

In connection with the foregoing side reactions and secondary reactions, it should be noted that all present data indicate that a true interpolymer of the olefin reactants is formed. Although the reaction mechanism involved is not completely understood, and it is to be understood that the invention is not to be restricted to any reaction mechanism, it does not appear that the excellent results obtained are attributable to separate polymerization of the short chain mono-olefin and of the long chain 1-olefin. It is most probable that wax-like material would be formed by a separate polymerization of long chain 1-olefin and the presence of such material would be indicated by a high pour point of the product. Inasmuch as the products have relatively low pour points, it is unlikely that any appreciable individual polymerization of the long chain 1-olefin occurs under the conditions of operation. Similarly, should any substantial portion of the short chain olefin polymerize separately, the products would have rather low viscosity indices. As emphasized above, however, the synthetic lubricants of this invention have high viscosity indices, of the order of 100 and higher. It is on this basis, then, that the products are considered to be true interpolymers.

Other reaction conditions to be considered in forming the lubricants contemplated herein are pressure and reaction time. The pressure to be used is not particularly critical. It may range from about 100 to about 10,000 pounds per square inch, or even higher. Increased pressure is desirable and, as expected, increased oil yields result. Pressures greater than about 500 per square inch are preferred.

Reaction time varies inversely with temperature. Satisfactory products and satisfactory yields of the same have been obtained with reaction times as short as one hour or less and as long as thirty hours. Preferably, the time is in the neighborhood of five to ten hours, at about 600° F. Most advantageous results are realized with a reaction time of from three to twenty hours at temperatures from about 600° F. to about 650° F. Test data also indicate that reasonable yields of products of comparatively high viscosity index may be obtained at temperatures of 750° F. to 800° F. with times of several minutes. These conditions are not advantageous, however, because the products have high pour points, and material which is not converted into oil is degraded into light fractions of a relatively low degree of unsaturation. The latter fractions, therefore, are undesirable as recycle stock. The viscosity index decreases sharply with prolonged exposure to these higher temperatures, namely, 750-800° F.

#### Examples

In order to illustrate the principles of this invention, the results of a series of typical, and non-limiting, condensations are set forth in tabular form in Table I below. These condensations were carried out in a rocking-type bomb (American Instrument Co.). In the case of hexa-

decene-1 and ethylene, for example, the bomb was charged with 224 parts by weight (1 molar proportion) of hexadecene-1. The atmosphere in the bomb was replaced with nitrogen and the bomb was then evacuated. Ethylene was next admitted from a cylinder. The bomb was then heated to the desired temperature for the desired length of time. During the run, ethylene was added several times. The total pressure drop was noted. The bomb was cooled and discharged. The contents of the bomb were vacuum topped to remove the more volatile non-viscous materials, and the product was filtered. To distinguish the condensation products from the distillate products thereof, the refined oils are identified as "residual oils." The latter term identifies the oils from which unreacted materials and products of intermediate boiling range have been separated.

It should be noted that the reaction times, recorded in "Time, Hours" in Table I, represent the time intervals during which the bomb was maintained at the desired temperature; and do not include the time intervals necessary to heat the

bomb and its contents to the desired temperature, nor include the time intervals necessary to cool the bomb after heat to the bomb has been discontinued. In general, about one and one half hours are required to raise the temperature from 60-80° F. to 600° F., and about three hours or more to cool thereafter to 60-80° F., in runs such as shown in Table I.

All of the tests and analyses to which the residual oils in Table I were subjected are well known standard tests. In this connection, it will be noted that the designation "N. N." refers to the neutralization number, which is a measure of the acidity of the oil; the designation "Br<sub>2</sub> No." refers to the bromine addition number, which is a measure of the unsaturation of the oil; the designation "Carbon Res." identifies the carbon residue, Ramsbottom determination; the designation "Vis., S. U. S. @ 210° F." refers to the viscosity at 210° F., in Saybolt Universal seconds as converted from kinematic determination; the abbreviation "V. I." represents viscosity index; "Means C chain" refers to the mean carbon chain length of the olefins charged.

**Table I**

| Run No.                               | 1                 | 2                 | 3                 | 4               | 5                 | 6              | 7              |
|---------------------------------------|-------------------|-------------------|-------------------|-----------------|-------------------|----------------|----------------|
| Short Chain Olefin                    | Ethylene          | Ethylene          | Ethylene          | Ethylene        | Ethylene          | Ethylene       | Propylene      |
| Parts by Weight                       | 35 <sup>A</sup>   | 34 <sup>A</sup>   | 26 <sup>A</sup>   | 24              | 67 <sup>A</sup>   | 16             | 102.           |
| Molar Proportions                     | 1.25              | 1.2               | 0.93              |                 |                   |                | 2.4.           |
| Long Chain Olefin                     |                   | Decene-1          | Decene-1          | Decene-1        | Hexadecene-1      | Hexadecene-1   |                |
| Parts by Weight                       |                   | 280               | 249               | 280             | 224               | 252            |                |
| Molar Proportions                     |                   | 2.0               | 1.8               | 2.0             | 1.0               | 1.1            |                |
| Other Olefins                         |                   |                   |                   |                 |                   |                |                |
| Parts by Weight                       |                   |                   |                   |                 |                   |                |                |
| Molar Proportions                     |                   |                   |                   |                 |                   |                |                |
| Mean C Chain                          | 2.                | 7.                | 7.4               | 10              | 6.1               | 16             | 3.             |
| Temperature, °F.                      | 610.              | 550               | 660               | 600             | 660               | 660            | 610.           |
| Time, Hours                           | 10.               | 10 <sup>A</sup>   | 9                 | 10 <sup>A</sup> | 10                | 11             | 10.            |
| Atmosphere                            | Evacuated         | Evacuated         | Evacuated         | N <sub>2</sub>  | Evacuated         | N <sub>2</sub> | N <sub>2</sub> |
| Max. Pressure, p. s. i.               | 2800              | 6800              | 2000              | 400             | 2300              | 200            | 1500.          |
| Cumulative Pressure Drop, p. s. i. g. | 1650 <sup>D</sup> | 2400 <sup>D</sup> | 1400 <sup>D</sup> | 75 <sup>D</sup> | 3100 <sup>D</sup> |                |                |
| Vacuum Distillate:                    |                   |                   |                   |                 |                   |                |                |
| Parts by Weight                       | 7.                | 244               | 143               | 205             | 89                | 74             |                |
| Yield, per cent <sup>F</sup>          | 20.               | 77.6              | 52                | 73              | 30.5              | 29.2           |                |
| Spec. Gravity                         |                   | 0.7491            | 0.7571            | 0.7479          | 0.7583            | 0.7883         |                |
| Br <sub>2</sub> No.                   | 90.3              | 90.7              | 82.9              | 102.7           | 35.9              | 48.3           |                |
| Residual Oil:                         |                   |                   |                   |                 |                   |                |                |
| Parts by Weight                       | 14                | 55                | 125               | 63              | 184               | 138            | 5.             |
| Yield, per cent <sup>F</sup>          | 40                | 17.2              | 45.4              | 22.5            | 63.1              | 54.8           | 4.9.           |
| Spec. Gravity                         | 0.8378            | 0.8418            | 0.8309            | 0.8309          | 0.8403            | 0.8368         | 0.7887.        |
| Br <sub>2</sub> No.                   | 25.0              | 10.8              | 22.5              | 16.6            | 12.2              | 12.8           | 62.8.          |
| N. N.                                 | 1.0               | 0.2               | 0.4               | 0.6             | 0.5               | 0.3            | 1.4.           |
| Refractive Index                      |                   |                   |                   |                 |                   |                |                |
| Carbon Res., Wt. per cent             | 52.77             | 62.46             | 40.85             | 44.43           | 47.94             | 50.47          | 30.            |
| Vis., S. U. S. @ 210° F.              | 115.4             | 125.3             | 135.4             | 143             | 138.2             | 146            |                |
| Pour Point, °F.                       | <-30.             | <-30.             | <-30.             | -25             | 15                | +75            | <-30.          |

| Run No.                               | 8                 | 9                | 10                | 11                | 12               | 13               | 14             |
|---------------------------------------|-------------------|------------------|-------------------|-------------------|------------------|------------------|----------------|
| Short Chain Olefin                    | Propylene         | Butene-1         | Isobutane         | Isobutene         |                  |                  |                |
| Parts by Weight                       | 612.              | 162              | 708               | 228               |                  |                  |                |
| Molar Proportions                     | 14.6              | 2.9              | 12.6              | 4.1               |                  |                  |                |
| Long Chain Olefin                     |                   |                  |                   |                   |                  |                  |                |
| Parts by Weight                       |                   |                  |                   |                   |                  |                  |                |
| Molar Proportions                     |                   |                  |                   |                   |                  |                  |                |
| Other Olefins                         |                   |                  |                   |                   |                  |                  |                |
| Parts by Weight                       |                   |                  |                   |                   |                  |                  |                |
| Molar Proportions                     |                   |                  |                   |                   |                  |                  |                |
| Mean C Chain                          | 3.                | 4                | 4                 | 5.3               | 400              | 200              | 200.           |
| Temperature, °F.                      | 650.              | 650              | 650               | 650               | 665              | 650              | 650.           |
| Time, Hours                           | 10.               | 9                | 10                | 10                | 10               | 9                | 20.            |
| Atmosphere                            | Evacuated         | Evacuated        | Evacuated         | Evacuated         | N <sub>2</sub>   | N <sub>2</sub>   | N <sub>2</sub> |
| Max. Pressure, p. s. i.               | 2400.             | 1600.            | 2325.             | 4100.             | 525              | 1150.            | 900.           |
| Cumulative Pressure Drop, p. s. i. g. | 1400 <sup>E</sup> | 900 <sup>E</sup> | 1075 <sup>E</sup> | 3475 <sup>E</sup> | 175 <sup>E</sup> | 250 <sup>E</sup> |                |
| Vacuum Distillate:                    |                   |                  |                   |                   |                  |                  |                |
| Parts by Weight                       | 132.              | 43               | 161               | 207               | 168              | 35               | 97.            |
| Yield, per cent <sup>F</sup>          | 21.6              | 26.5             | 22.8              | 45.6              | 42               | 17.5             | 48.5.          |
| Spec. Gravity                         |                   | 0.8040           | 0.8104            | 0.7990            |                  | 0.8067           | 0.7945.        |
| Br <sub>2</sub> No.                   |                   | 49.3             | 52.0              | 55.8              |                  | 88.7             | 79.4.          |
| Residual Oil:                         |                   |                  |                   |                   |                  |                  |                |
| Parts by Weight                       | 52.               | 5                | 20                | 63                | 179              | 3                | 21.            |
| Yield, per cent <sup>F</sup>          | 8.5               | 3.0              | 2.8               | 13.9              | 44.8             | 1.5              | 10.5.          |
| Spec. Gravity                         | 0.9705            | 0.8462           | 0.8822            | 0.8473            | 0.8448           |                  | 0.8607.        |
| Br <sub>2</sub> No.                   | 46.9              | 28.9             | 44.7              |                   | 22.1             | 51.7             | 52.1.          |
| N. N.                                 | 1.3               | 10               |                   |                   |                  | 1.95             | 1.0.           |
| Refractive Index                      |                   |                  |                   |                   |                  |                  |                |
| Carbon Res., Wt. per cent             | 43.6              | 37.98            | 43.79             | 43.83             | 41.95            | 34.04            | 37.09.         |
| Vis., S. U. S. @ 210° F.              | -85               | 35.8             | <0                | 84.0              | 123.0            | 51.7             | 34.8.          |
| Pour Point, °F.                       | -25               | <-30             | <-30              | <-30              | <-30             | <-30             | <-30.          |

Table I—Continued

| Run No.                               | 15                | 16                | 17             | 18               | 19                                   | 20                         |
|---------------------------------------|-------------------|-------------------|----------------|------------------|--------------------------------------|----------------------------|
| Short Chain Olefin                    | Isobutene         | Isobutene         |                | Hexene-1         |                                      |                            |
| Parts by Weight                       | 228               | 208               |                | 84               |                                      |                            |
| Molar Proportions                     | 4.1               | 3.7               |                | 1.0              |                                      |                            |
| Long Chain Olefin                     | Hexadecene-1      |                   |                | Hexadecene-1     |                                      |                            |
| Parts by Weight                       | 224               |                   |                | 224              |                                      |                            |
| Molar Proportions                     | 1.0               |                   |                | 1.0              |                                      |                            |
| Other Olefins                         |                   | Mixed Olefins     | Pentene-2      |                  | C <sub>3</sub> -Polymer <sup>a</sup> | Mixed Olefins <sup>c</sup> |
| Parts by Weight                       |                   | 200               | 200            |                  | 172                                  | 200                        |
| Molar Proportions                     |                   | 0.13 <sup>b</sup> | 2.9            |                  |                                      | C <sub>4</sub> , 2.        |
| Mean C Chain                          | 6.3               | 4.4               | 5              | 11               | 9                                    | 610.                       |
| Temperature, °F                       | 650               | 650               | 605            | 600              | 640                                  | 534.                       |
| Time, Hours                           | 10                | 10                | 10             | 10               | 9                                    | N <sub>2</sub>             |
| Atmosphere                            | Evacuated         | Evacuated         | N <sub>2</sub> | N <sub>2</sub>   | N <sub>2</sub>                       | N <sub>2</sub>             |
| Max. Pressure, p. s. i.               | 4800              | 3500              | 1725           | 600              | 600                                  | 400                        |
| Cumulative Pressure Drop, p. s. i. g. | 4126 <sup>e</sup> | 2350 <sup>e</sup> |                | 100 <sup>d</sup> | 100 <sup>d</sup>                     | 50. <sup>d</sup>           |
| Vacuum Distillate:                    |                   |                   |                |                  |                                      |                            |
| Parts by Weight                       | 178               | 250               |                | 101              |                                      | 48.                        |
| Yield, per cent <sup>f</sup>          | 39.3              | 61.2              |                | 32.8             |                                      | 24.                        |
| Spec. Gravity                         | 0.8003            | 0.8478            |                | 0.7857           |                                      | 0.7665.                    |
| Br. No.                               | 49.1              | 43.9              |                | 67.7             |                                      | 90.7.                      |
| Residual Oil:                         |                   |                   |                |                  |                                      |                            |
| Parts by Weight                       | 192               | 51                | 5              | 143              | 3                                    | 68.                        |
| Yield, per cent <sup>f</sup>          | 42.5              | 12.8              | 2.5            | 46.4             | 1.74                                 | 34.                        |
| Spec. Gravity                         | 0.8368            | 0.9440            | 0.7778         | 0.8270           |                                      | 0.8403.                    |
| Br. No.                               |                   | 18.4              | 35.8           | 21.6             |                                      | 27.4.                      |
| N. N.                                 |                   |                   | 1.2            | 0.2              |                                      | 0.1.                       |
| Refractive Index                      |                   |                   |                |                  |                                      |                            |
| Carbon Res., Wt. per cent             | 0.02              | 1.1               |                |                  |                                      |                            |
| Vis., S. U. S. @ 210° F               | 42.41             | 73.23             | (N)            | 38.77            |                                      | 41.98.                     |
| V. I.                                 | 132.6             | <0                | (5)            | 138.0            |                                      | 137.3.                     |
| Pour Point, °F                        | 10                | -15               | <-80           | -15              |                                      | -30.                       |

<sup>a</sup> Ethylene reacting, calculated from weight of liquid product in bomb.<sup>b</sup> Mixed olefins; boiling range 570-620° F.; Br. No. 10; average carbon chain about 16; obtained from cracking of heavy gas oil. Low bromine number indicates only about 15 per cent olefins, remainder paraffins.<sup>c</sup> Mixed olefins; boiling range 44-225° C.; average carbon chain about 8; obtained from thermally cracked paraffin wax.<sup>d</sup> At approximately 600° F.<sup>e</sup> At approximately 650° F.<sup>f</sup> Based upon total charge of olefins shown.<sup>g</sup> Propylene polymer, predominantly a mixture of nonenes, low in alpha olefin content.<sup>h</sup> Approximately 30 sec. S. U. @ 100° F.<sup>i</sup> Considering only 30 g. olefins of C<sub>4</sub> range.<sup>j</sup> V. I. off-scale—cannot be calculated significantly for very low viscosity product.

From the data set forth in Table I above, several observations may be made. Run 1 indicates that a synthetic oil of excellent quality may be prepared by thermal treatment of ethylene. Runs 2, 3 and 5 reveal that mixtures of ethylene and long chain 1-olefins, namely, decene-1 and hexadecene-1, may be converted thermally to outstanding viscous oils, the olefins being so proportioned on a molar basis that the mean carbon chain length ranges from 6.1 to 7.4. Each of the oils formed in Runs 2, 3 and 5 is characterized by a V. I. substantially above 100. Run 4 shows an oil obtained by thermal conversion of decene-1, such an oil being shown for purposes of comparison with the oils of Runs 2 and 3; Run 4 is typical of those described in the aforesaid parent application. Run 5 shows an excellent oil of this invention, the oil being derived from ethylene and hexadecene-1. In comparison, the oil obtained from hexadecene-1 alone, in Run 6, has a most satisfactory viscosity index but an excessively high pour point.

Demonstrating that thermal conversion of short chain olefins alone results in low yields of viscous products of poor quality are Runs 7, 8, 9 and 10. For example, the yields range from 2.8% to 8.5%, and the viscosity indices range from -85 to 35.8. Run 11 illustrates an oil having a V. I. of only 84; the mean carbon chain length of the olefin mixture was only 5.3, which is below the lower limit of 6.

Run 12 is typical of the oils of the aforesaid parent application.

Runs 13 and 14 show that olefins of intermediate chain length having other than a normal, alpha character do not form desirable viscous oils when converted thermally.

Run 15 shows an oil contemplated herein; the oil is derived from isobutene and hexadecene-1.

Run 16 is unsatisfactory because long-chain olefins were not available in sufficient amount or purity, and because the mean carbon chain length of the olefin mixture was only 4.4.

Run 17 shows the unsatisfactory oil obtained in low yield from pentene-2 which, of course, is not an alpha olefin.

Run 18 shows an excellent oil obtained from a mixture of hexene-1 and hexadecene-1 in proper proportion.

Run 19 involves thermal conversion of mixed nonenes, low in alpha olefin content, with the formation of only a small quantity of residual oil; such is not contemplated herein.

Run 20 is also illustrative of the oils of the aforesaid parent application.

As will be evident from the data presented above in Table I, the condensation products of this invention are highly desirable lubricants per se. They are also of considerable value as blending agents for other lubricating oils. In view of the inherent stability of the synthetic oils, they impart stability to the oils with which they are blended. So also, they impart desirable viscosity index (V. I.) and pour point characteristics to the oils in combination therewith, for, as indicated above, they have advantageous viscosity index and pour point properties. In short, the synthetic oils find utility in "upgrading" other lubricants. Typical oils with which the synthetic oils may be blended are mineral oils such as are normally used in internal combustion and turbine engines. When so blended, the synthetic oils may comprise the major proportion of the final blended oil, or may even comprise a minor proportion thereof.

One or more of the individual properties of the synthetic lubricants of this invention may be further improved by incorporating therewith a small, but effective amount, of an addition agent such as an anti-oxidant, a detergent, an extreme pressure agent, a foam suppressor, a viscosity index (V. I.) improver, etc. Representative anti-oxidants are phenols, catechols, amines including phenylene diamines, etc. Typical detergents which may be so used are metal salts of alkyl-substituted aromatic sulfonic or carboxylic acids,

as illustrated by diwax benzene barium sulfonate and barium phenate, barium carboxylate of a wax-substituted phenol carboxylic acid. Extreme pressure agents are well-known; illustrating such materials are numerous chlorine and/or sulfur containing compositions, one such material being a chloronaphtha xanthate. Silicones, such as dimethyl silicone, may be used to illustrate foam suppressing compositions. Viscosity index improving agents which may be used are typified by polypropylenes, polyisobutylenes, polyacrylate esters, and the like.

Contemplated also as within the scope of this invention is a method of lubricating relatively moving surfaces by maintaining therebetween a film consisting of any of the aforesaid oils.

It is to be understood that the foregoing description and representative examples are non-limiting and serve to illustrate the invention, which is to be broadly construed in the light of the language of the appended claims.

We claim:

1. The method for preparing a viscous oil, which comprises: thermally and non-catalytically condensing, at a temperature between about 500° F. and about 750° F. for a period of time from about twenty hours to about one hour, respectively, an olefin mixture consisting essentially of a short chain mono-olefin having from two to six carbon atoms per molecule and a long-chain normal, alpha mono-olefin having from ten to thirty carbon atoms per molecule; said short chain and long chain olefins being reacted in such molar proportions that the mean value of the olefin chain length in the olefin mixture is from about six to about twelve carbon atoms.

2. The method for preparing a viscous oil, which comprises: thermally and non-catalytically condensing, at a temperature between about 600° F. and about 700° F. for a period of time from about five to about ten hours at 600° F. to about one hour at 700° F., respectively, an olefin mixture consisting essentially of a short chain mono-olefin having from two to six carbon atoms per molecule and a long chain normal, alpha mono-olefin having from ten to thirty carbon atoms per molecule; said short chain and long chain olefins being reacted in such molar proportions that the mean value of the olefin chain length in the olefin mixture is from about six to about twelve carbon atoms.

3. The method for preparing a viscous oil, which comprises: thermally and non-catalytically condensing, at a temperature between about 500° F. and about 750° F. for a period of time from about twenty hours to about one hour, respectively, an olefin mixture consisting essentially of a short chain mono-olefin having from two to six carbon atoms per molecule and a long chain normal, alpha mono-olefin having from twelve to twenty carbon atoms per molecule; said short chain and long chain olefins being reacted in such molar proportions that the mean value of the olefin chain length in the olefin mixture is about ten carbon atoms.

4. The method for preparing a viscous oil, which comprises: thermally and non-catalytically condensing, at a temperature between about 500° F. and about 750° F. for a period of time from about twenty hours to about one hour, respectively, an olefin mixture consisting essentially of a short chain normal, alpha mono-olefin having from two to six carbon atoms per molecule and a long chain normal, alpha mono-olefin having from twelve to twenty carbon atoms per molecule;

said short chain and long chain olefins being reacted in such molar proportions that the mean value of the olefin chain length in the olefin mixture is from about six to about twelve carbon atoms.

5. A viscous oil characterized by a viscosity index of at least about 100 and by a low pour point, and obtained by: thermally and non-catalytically condensing, at a temperature between about 500° F. and about 750° F. for a period of time from about twenty hours to about one hour, respectively, an olefin mixture consisting essentially of a short chain mono-olefin having from two to six carbon atoms per molecule and a long chain normal, alpha mono-olefin having from ten to thirty carbon atoms per molecule; said short chain and long chain olefins being reacted in such molar proportions that the mean value of the olefin chain length in the olefin mixture is from about six to about twelve carbon atoms.

6. A viscous oil characterized by a viscosity index of at least about 100 and by a low pour point, and obtained by: thermally and non-catalytically condensing, at a temperature between about 600° F. and about 700° F. for a period of time from about five to about ten hours at 600° F. to about one hour at 700° F., respectively, an olefin mixture consisting essentially of a short chain mono-olefin having from two to six carbon atoms per molecule and a long chain normal, alpha mono-olefin having from ten to thirty carbon atoms per molecule; said short chain and long chain olefins being reacted in such molar proportions that the mean value of the olefin chain length in the olefin mixture is from about six to about twelve carbon atoms.

7. A viscous oil characterized by a viscosity index of at least about 100 and by a low pour point, and obtained by: thermally and non-catalytically condensing, at a temperature between about 500° F. and about 750° F. for a period of time from about twenty hours to about one hour, respectively, an olefin mixture consisting essentially of a short chain mono-olefin having from two to six carbon atoms per molecule and a long chain normal, alpha mono-olefin having from twelve to twenty carbon atoms per molecule; said short chain and long chain olefins being reacted in such molar proportions that the mean value of the olefin chain length in the olefin mixture is about ten carbon atoms.

8. A viscous oil characterized by a viscosity index of at least about 100 and by a low pour point, and obtained by: thermally and non-catalytically condensing, at a temperature between about 500° F. and about 750° F. for a period of time from about twenty hours to about one hour, respectively, an olefin mixture consisting essentially of a short chain normal, alpha mono-olefin having from two to six carbon atoms per molecule and a long chain normal, alpha mono-olefin having from twelve to twenty carbon atoms per molecule; said short chain and long chain olefins being reacted in such molar proportions that the mean value of the olefin chain length in the olefin mixture is from about six to about twelve carbon atoms.

9. A viscous oil characterized by a viscosity index of at least about 100 and by a low pour point, and obtained by: thermally and non-catalytically condensing, at about 660° F. for about ten hours, an olefin mixture consisting essentially of ethylene and hexadecene-1; said ethylene and hexadecene-1 being reacted in such molar proportions that the mean value of the olefin chain

11

length in the olefin mixture is about six carbon atoms.

10. A viscous oil characterized by a viscosity index of at least about 100 and by a low pour point, and obtained by: thermally and non-catalytically condensing, at about 650° F. for about ten hours, an olefin mixture consisting essentially of isobutene and hexadecene-1; said isobutene and hexadecene-1 being reacted in such molar proportions that the mean value of the 10 olefin chain length in the olefin mixture is about six carbon atoms.

11. A viscous oil characterized by a viscosity index of at least about 100 and by a low pour point, and obtained by: thermally and non-catalytically condensing, at about 660° F. for

12

about ten hours, an olefin mixture consisting essentially of hexene-1 and hexadecene-1; said hexene-1 and hexadecene-1 being reacted in such molar proportions that the mean value of the olefin chain length in the olefin mixture is about eleven carbon atoms.

FRANCIS M. SEGER.

ALEXANDER N. SACHANEN.

## REFERENCES CITED

The following references are of record in the file of this patent:

## UNITED STATES PATENTS

15 Number Name Date  
2,315,080 Reid Mar. 30, 1943